

# UNITED STATES PATENT OFFICE.

ROBERT B. COREY, OF EDGEWOOD PARK, PENNSYLVANIA.

## CEMENTING OR CASE-HARDENING MATERIAL.

1,211,093.

Specification of Letters Patent.

Patented Jan. 2, 1917.

No Drawing.

Application filed March 29, 1916. Serial No. 87,515.

To all whom it may concern:

Be it known that I, ROBERT B. COREY, a citizen of the United States, residing at Edgewood Park, in the county of Allegheny and State of Pennsylvania, have invented certain new and useful Improvements in Cementing or Case-Hardening Materials, of which the following is a specification.

My invention relates to the art of cementation or case-hardening of iron or steel and more particularly to materials used in such cementing or case-hardening processes.

The objects of my invention are to increase the rapidity of the penetration of the carbon into the iron or steel to be treated and to accomplish this result by the dry, packing process without the necessity of expensive or complicated apparatus.

My invention consists of a mixture of carbon or carbonaceous material with a material which acts to quickly transfer the carbon to the surface of the iron or steel and to accomplish this transfer so quickly and effectively that a further rapid transfer of carbon takes place between the molecules of the heated iron or steel, resulting in a thick layer of highly carbonized metal upon the surface of the material so treated, the thickness of the layer depending upon the duration of the treatment and the temperature to which the cementing material and the iron or steel parts are subjected.

More particularly, my invention consists in the use of a mixture of carbon or carbonaceous material and oxid of magnesium.

In carrying out my invention, the carbon or carbonaceous material is preferably finely divided and the oxid of magnesium is thoroughly mixed therewith. In practice, I usually add to the carbonaceous material about ten per cent. by weight of oxid of magnesium but I have found that the percentage of magnesium oxid present in the mixture is not essential to its action in the carbonization of the iron or steel and that, throughout the duration of the cementing or case-hardening process, the said percentage is continually changing on account of the absorption of carbon by the iron or steel, and other chemical changes that may take place in the heated

furnace. When the carbon becomes exhausted the remaining oxid of magnesium may be added to fresh carbon or carbonaceous material, thus reducing the cost of the cementing material to the minimum.

It is obvious that, instead of using oxid of magnesium for this process, the carbonate of magnesium may be used, as, upon the application of heat, the carbonate of magnesium will be decomposed, gaseous oxid of carbon being liberated and the oxid of magnesium remaining, or both carbonate of magnesium and oxid of magnesium may be mixed with the carbon to form the cementing material.

I have found that the use of magnesium-containing compounds as above mentioned, in the cementing or case-hardening process, greatly reduces the length of time necessary to produce a carbonized layer of iron or steel of any desired depth.

I am aware that magnesium sulfate has been used in cementation processes. Upon heating the sulfate is decomposed and sulfurous gases are generated. Magnesium sulfate is very objectionable for this purpose, as it is found that the sulfurous gases liberated in contact with highly heated iron are partially absorbed, producing a layer of sulfurous steel which is very weak and brittle, whereas, if there is no sulfur present the resulting steel will be both strong and tough, it being suitable for tools, automobile gears and steel structures that are required to withstand severe shocks. I, therefore, confine myself to the use of magnesium compounds that have no sulfur in their composition.

I do not desire to limit myself to the exact materials and proportions above specified, but aim in the appended claims to cover all modifications which are within the scope of my invention.

What I claim as new and desire to secure by Letters Patent of the United States is—

1. A cementing or case hardening material consisting essentially of carbonaceous material with not less than ten per cent. of oxid of magnesium.
2. A cementing or case-hardening mate-

rial consisting essentially of carbonaceous material with not less than ten per cent. of a compound reducible by heat to oxid of magnesium.

3. A cementing or case-hardening material consisting essentially of carbonaceous material with oxid of magnesium and carbonate of magnesium, the total weight of the said magnesium compounds being not

less then ten per cent. of the weight of the 10 said cementing material.

In witness whereof I have set my hand this 27th day of March, 1916.

**ROBERT B. COREY.**

Witnesses:

**FRED B. COREY,**  
**M. MENDEL.**